

1,175,611.

G. S. COX.

HAIRCLOTH FABRIC AND PROCESS OF MAKING SAME.  
APPLICATION FILED JULY 20, 1915.

Patented Mar. 14, 1916.



FIG. 2.



FIG. 1.



WITNESS:

Prof. R. Kitchell

INVENTOR

George S. Cox  
by Frank J. Besser

ATTORNEY.

# UNITED STATES PATENT OFFICE.

GEORGE S. COX, OF PHILADELPHIA, PENNSYLVANIA.

## HAIRCLOTH FABRIC AND PROCESS OF MAKING SAME.

1,175,611.

Specification of Letters Patent. Patented Mar. 14, 1916.

Application filed July 20, 1915. Serial No. 40,815.

*To all whom it may concern:*

Be it known that I, GEORGE S. Cox, a citizen of the United States, residing at Philadelphia, county of Philadelphia, and State 5 of Pennsylvania, have invented a new and useful Improvement in Haircloth Fabric and Processes of Making Same, of which the following is a full, clear, and exact description, reference being had to the accompanying drawings, which form a part of 10 this specification.

Probably the only objection to the employment of hair-cloth as a stiffener for clothing is the tendency of the individual hairs to 15 work out of the fabric and project through the garment. These projecting ends of hair-cloth are unsightly as well as unpleasant to the touch, and the wearer of the garment usually pulls out the lengths of hair 20 whose ends project. While this results often in substantial loss of stiffness, the main objection is usually the offense to touch and sight before mentioned.

The main object of the invention is to so 25 treat the fabric as to eliminate any tendency of the hairs to work out and at the same time not deleteriously affect either the desired stiffness or flexibility of the hair-cloth.

Another object of the invention is to improve, in general, the appearance, quality 30 and efficiency of the cloth.

The invention is applicable either to cloth in which the weft is composed entirely of hair or to cloth in which the weft is composed 35 partly of hair and partly of linen, cotton or other textile yarn. I have illustrated my invention as applied to the ordinary plain-weave hair-cloth of commerce.

Figure 1 is a diagram of an apparatus 40 which may be used to carry out my process. Fig. 2 is a diagrammatic cross-sectional view of my improved fabric after treatment.

It will be understood that my process is 45 not dependent for its execution upon any particular mechanism and indeed may be carried out, less economically, by hand. It may also be stated that while the finished product is capable of fairly accurate description, it can be illustrated only with 50 some approximation to the actual condition, and Fig. 2 is to be considered, therefore, as to a certain extent an ideal or picture diagram of the completed article of manufacture.

The ordinary hair-cloth fabric, which I

have elected to use as an illustration of a fabric to which the invention may be applied, consists of a plain up-and-down weave in which the warp threads *y*, *y*, are 60 of cotton and the weft *z* of hair, there being one pick of hair in each shed of warp. This fabric, after it is woven, is caused to travel through a bath of rubber cement. While I prefer to employ rubber cement, the invention is not limited to the employment of any particular composition, and the term 65 "cement" where hereinafter used, is intended to include any substance which is capable of being substituted for the rubber 70 cement and which will act in a similar manner. The receptacle *a* for cement is shown at the left-hand end of Fig. 1.

*b*, *b*, *b* represent guide rollers for directing the cloth into and through the receptacle. 75

When the cloth emerges from the bath it is coated with the cement, which, however, has not, perhaps, thoroughly yet permeated the interstices of the fabric; and furthermore, an excess of cement is carried by the fabric. The fabric is therefore passed through a pair of rolls *c*, which may be roughly called squeeze rolls, the function of which is to force the cement thoroughly 80 into the interstices of the fabric and to remove all cement in excess of that which it is desired to retain in the goods. The degree of pressure upon the fabric may be regulated as experience dictates. The fabric is then fed over guide rolls *d*, *d*, etc. through a drier *e*, which reduces the softness and stickiness of the cement, whence the fabric is led through one or more pairs of rolls *f*, *f*, which have a further consolidating action upon the cement. The operation need not be a continuous one, and I have indicated this lack of continuity by illustrating the fabric in dotted lines 85 between the rolls *f* and *f*; it being understood 90 that, at this point in the process, the fabric may be removed and allowed to dry under natural or artificial conditions for any not too prolonged length of time. By means of guide rolls *g*, *g*, the fabric is then fed, preferably in an upward direction, between a pair of brushes *h*. These brushes are located immediately below hoppers *i*, which contain powdered talc, soapstone, sulfur or any other ingredient, preferably in 95 powdered form, that will perform the same function. The brushes *h* rotate in a direc-

100  
105  
110

tion opposite to that of the travel of the cloth and serve to cover the cementitious surface of the cloth with a thin coating of the powder. Beyond the upper guide roll 5 *g* the brushes pass between a pair of calender rolls *j*, which serve to press the powder into the body of cement near its surface and finish and harden such surface. Beyond the calendar rolls *j* the cloth passes between a pair of brushes *m*, which, like brushes *h*, rotate oppositely to the direction of travel of the rolls. These brushes remove the loose excess of powder remaining on the surface of the cloth. Rolls *n*, *n*, are merely feed 10 rolls which draw the fabric through the coating mechanism described. The treatment of the hair-cloth is then practically completed, although it may be further dried.

In place of dusting the cement-impregnated cloth with powder it may be coated with a liquid veneer as, for example, starch and water, but the product is not quite so satisfactory.

The result of the described treatment is 25 to produce the fabric diagrammatically illustrated in Fig. 2, in which the weave is permeated, more or less completely, by a cementitious substance having a comparatively hard, smooth, thin surface *w* and a 30 comparatively soft yielding interior *x*. The comparatively soft interior insures the desired maintenance of the flexibility of the cloth and binds the hairs securely in position while the hard smooth surface prevents 35 any superficial stickiness and maintains the interior in the relatively soft condition best adapted to hold the hairs from longitudinal movement.

In using the term "hair-cloth" in the 40 claims I desire it to be understood as comprising the ordinary hair-cloth of commerce or any variations thereof presenting, when untreated, the conditions which it is the purpose of my invention to eliminate.

Having now fully described my invention, what I claim and desire to protect by Letters Patent is:

1. As a new article of manufacture, hair 50 cloth and material applied thereto providing an impregnating and relatively soft cementitious interior and a relatively hard surface.

2. As a new article of manufacture, hair 55 cloth and material applied thereto providing an impregnating and relatively soft cementitious interior and a relatively smooth non-sticky surface.

3. As a new article of manufacture, hair 60 cloth impregnated with a cementitious substance and a substance applied to, and serving to superficially harden, the relatively soft cementitious substance.

4. As a new article of manufacture, hair 65 cloth impregnated with a cementitious sub-

stance and another substance superficially pressed into the cementitious substance and uniting therewith to modify the exposed surface of the impregnating substance.

5. As a new article of manufacture, hair 70 cloth impregnated with a cementitious substance and another substance superficially pressed into the cementitious substance and uniting therewith to render the exposed surface of the impregnating substance relatively smooth and non-sticky. 75

6. As a new article of manufacture, hair cloth impregnated with a cementitious substance and a coating of a powdered solid substance applied to the opposite faces 80 thereof.

7. As a new article of manufacture, hair cloth impregnated with a cementitious substance and a powdered solid substance superficially consolidated with the cementitious substance. 85

8. As a new article of manufacture, hair cloth impregnated with a cementitious body in a relatively soft adhesive condition and superficial layers composed of said cementitious substance and a powdered solid impregnated therewith and providing a relatively smooth and hard protective coating. 90

9. As a new article of manufacture, hair cloth impregnated with rubber cement and a substance applied to, and serving to superficially harden, the relatively soft cement. 95

10. As a new article of manufacture, hair cloth impregnated with rubber cement and a substance applied to the surface of 100 the cemented fabric and rendering it relatively smooth and non-sticky.

11. As a new article of manufacture, hair cloth impregnated with rubber cement having a coating of powdered solid embedded therein. 105

12. As a new article of manufacture, hair cloth impregnated with rubber cement having an embedded coating of talc.

13. The process of finishing hair cloth 110 which consists in impregnating the same with a cementitious substance in solution and adapted to still present when dried an adhesive surface, then drying the cemented fabric, and then coating both surfaces of 115 the same with a hardening and smoothening substance.

14. The process of finishing hair cloth which consists in impregnating the same with a cementitious substance in solution 120 and adapted to still present when dried an adhesive surface, then drying the cemented fabric, and then coating both surfaces of the same with a powdered solid, and then compressing the same to cause the powdered solid to superficially impregnate the treated fabric. 125

15. The process of finishing hair cloth which consists in applying thereto a cementitious substance in solution and adapted 130

to still present when dried an adhesive surface, then subjecting the fabric to pressure to effect more thorough impregnation by, and removal of excess of, the cementitious substance, drying the cemented fabric, and coating both surfaces of the cemented fabric to harden and smoothen the same.

16. The process of finishing hair cloth which consists in applying thereto a cementitious substance in solution and adapted to still present when dried an adhesive surface, subjecting the fabric to pressure to effect a more thorough impregnation by and removal of excess of, the cementitious substance, drying the cemented fabric, coating

both surfaces of the same with a powdered solid, and compressing the cemented fabric to superficially impregnate the same with the powdered solid.

17. The process of finishing hair cloth 20 which consists in impregnating the same with rubber cement, then drying the cemented fabric, and then coating the surface of the same with a hardening and smoothening substance.

In testimony of which invention, I have hereunto set my hand, at Philadelphia, on this 10th day of July, 1915.

25

GEORGE S. COX.